

## UNITED STATES PATENT OFFICE.

THOMAS MIDGLEY, JR., OF DAYTON, OHIO, ASSIGNOR, BY MESNE ASSIGNMENTS, TO GENERAL MOTORS CORPORATION, OF DETROIT, MICHIGAN, A CORPORATION OF DELAWARE.

## METHOD AND MEANS FOR USING LOW-COMPRESSION FUELS.

No Drawing.

Application filed September 18, 1923. Serial No. 663,495.

*To all whom it may concern:*

Be it known that I, THOMAS MIDGLEY, Jr., a citizen of the United States of America, residing at Dayton, county of Montgomery, 5 and State of Ohio, have invented certain new and useful Improvements in Methods and Means for Using Low-Compression Fuels, of which the following is a full, clear, and exact description.

10 This invention relates to the art of suppressing a fuel knock when a combustible gaseous mixture containing a low compression fuel such, for example, as kerosene and gasoline is burned under a relatively 15 high pressure. The principal object of this invention is to employ tellurium compounds to suppress the fuel knock.

This application is a continuation in part 20 of my copending application, Serial No. 553,270, filed April 15, 1922.

Kerosene has a critical compression pressure of about 55 pounds. The critical compression pressure of gasoline varies from about 75 pounds for the commoner forms 25 now marketed, to about 125 pounds for "aviation gasoline" employed in airplane engines. These fuels are termed low compression fuels. When the vapors of any one of them is mixed with air, compressed 30 to a compression pressure in excess of the normal critical compression pressure of the fuel, and burned, as in an internal-combustion engine, a fuel knock is produced.

I have found that vapors of tellurium 35 compounds added to the fuel-air mixture suppress this fuel knock and permit an increase in the engine compression pressure with a normal burning characteristic of the fuel.

40 By way of an example of one method of carrying out my invention, I dissolve 5 c. c. of diethyl telluride  $\text{Te}(\text{C}_2\text{H}_5)_2$  in 1 gallon of gasoline having a normal critical compression pressure of about 75 pounds. This 45 solution or high compression fuel is fed through a carburetor into the cylinder of an internal-combustion engine having a

compression pressure of about 100 pounds, the solution being vaporized and mixed with air as is common practice in engine operation. The gaseous high compression fuel is ignited and the engine operated without a fuel knock. The gasoline forms the fuel base and the tellurium compound increases the critical compression pressure of this 55 base.

This process may be varied by changing the proportions according to the increase in critical compression pressure desired and by using other tellurium compounds in place of 60 the diethyl telluride. Among the compounds which I have successfully employed are other alkyl compounds including dipropyl and dimethyl telluride, and diphenyl telluride.

65 I prefer to employ the tellurium compounds which are soluble in the fuel to promote the mixing of the two. Blending agents may be employed if the tellurium compound does not dissolve readily in the 70 fuel. The compound may be added to the fuel-air mixture just before the latter is burned.

I claim:

1. A composition of matter comprising a 75 low compression fuel; and a volatile tellurium compound incorporated therein and adapted to increase the critical compression pressure of the fuel.

2. A composition of matter comprising a 80 low compression fuel, such as kerosene or gasoline; and a volatile alkyl compound of tellurium incorporated homogeneously therein and adapted to increase the critical compression pressure of the fuel.

85 3. A composition of matter comprising a low compression fuel; and a volatile ethyl compound of tellurium incorporated therein.

4. A composition of matter comprising 90 gasoline; and diethyl telluride.

In testimony whereof I hereto affix my signature.

THOMAS MIDGLEY, JR.